

## UNITED STATES PATENT OFFICE.

MONROE LAWRENCE PATZIG, OF DES MOINES, IOWA.

## BLOCK FOR PAVING AND THE LIKE AND PROCESS FOR MAKING THE SAME.

No Drawing.

Application filed August 27, 1924. Serial No. 734,544.

*To all whom it may concern:*

Be it known that I, MONROE L. PATZIG, a citizen of the United States, and a resident of Des Moines, in the county of Polk and

5 State of Iowa, have invented a certain new and useful Block for Paving and the like and Process for Making the Same, of which the following is a specification.

My invention has to do with a block or 10 brick peculiarly adapted for use in paving and other places where the block is subjected to heavy traffic and vibration and is or is not constantly subjected to the weather.

The purpose of my invention is to provide 15 such a block, which will have all the advantages of and be superior to sheet asphalt, but which utilizes natural asphaltic rock, rather than mixtures of asphalt or tar, sand, dust and rock, thereby utilizing material 20 available in this country and reducing the cost of the product, and which can be made in the factory and transported to the job in convenient form for use.

A further object is to provide such a 25 block and process for producing such a block, which will have homogeneity, resiliency and toughness, thus making it peculiarly adaptable for paving.

There are generally speaking several types 30 of paving in which asphalt is used, sheet asphalt, asphaltic concrete, and asphalt blocks.

In sheet asphalt, there is employed a 35 mixture of asphalt, dust and sand. The mixture is accomplished in a plant and is dumped, spread and stamped or rolled on the street.

This type of paving has the disadvantage 40 of requiring that the material be transported to the place of installation and that many different labor operations must there be performed. My blocks are made in the factory. Labor cost is cheaper and more uniform, high grade product can be produced. The number of operations on the 45 job and the labor of laying is much less.

In asphaltic concrete (fine aggregate), the same materials as are used in the making of sheet asphalt are employed with the 50 addition of rock of a variety of sizes up to one-half or three-quarters of an inch in greatest diameter, and the paving is prepared and laid on the job as in the case of sheet asphalt with similar disadvantages.

55 In asphaltic concrete (coarse aggregate), the same ingredients are used as in asphaltic

concrete with the addition of rock up to one inch or one and one-half inches in size, and the paving is prepared and laid on the job similar to sheet asphalt. 60

Actual experience, especially under heavy traffic conditions has demonstrated that sheet asphalt makes the best and most lasting paving. The paving with the larger sizes of rock deteriorates more rapidly and develops cracks and holes more extensively. 65

There is another type of asphalt pavement (patented), which may be the same as sheet asphalt and asphaltic concrete, with the addition of copper sulphate to the melted asphalt. 70

Still another type utilizes earth, clay or natural sandy soils mixed with asphalt.

Rock asphalt, such as the Kentucky rock asphalt and Uvalde rock asphalt are ground 75 and used in constructing pavements by being spread and rolled.

Asphalt blocks have been prepared and used, but so far as I have been able to ascertain, none have been employed, having 80 the same ingredients and qualities, or the same method of preparation as mine.

The greatest fault with all asphalt pavements is due to lack of uniformity. Lack of 85 uniformity is due to compounding batches of asphalt, due to variations of mineral aggregate, due to variations in weighing, due to variations in temperatures, due to variations in mixing, due to variations in spreading, due to variations in thickness and due 90 to variations in compressing.

With mixtures containing large particles of stone, uniformity becomes more difficult and the strain upon the cementitious material, asphalt, is greater. Such mixtures 95 are more apt to disintegrate on account of hammering action on the pavement fracturing the stone particles and forming pits, then holes.

Neither of the above-described methods 100 of producing asphalt pavements nor in the present mode of making asphalt blocks are the particles contained therein thoroughly impregnated with cementitious material, asphalt. 105

For this reason, I have utilized certain asphalt rock.

Asphalt rock is thoroughly impregnated with asphalt and the particles obtained by grinding are impregnated with asphalt. 110

In the other forms of pavement above referred to, it is not possible to get the uni-

formity of compounding asphalts, blending mineral aggregate, weighing, temperature, mixing, spreading, thickness and compressing, that I will be able to secure in my 5 process and materials.

In the case of asphalt block, as now manufactured, I will be able to improve upon same by utilizing thoroughly impregnated material and eliminating larger particles of 10 stone, thereby securing more uniformity and malleability.

In preparing my blocks, I employ natural asphaltic rock, ground, heated and pressed to shape. This rock affords both the cementitious material and the mineral 15 material.

I find that a block of maximum efficiency for the heavy duty of paving must have certain qualities that are secured only by 20 careful selection and preparation of the ingredients. Such a block must have great durability and therefore must have to a high degree, homogeneity or uniformity of mass, uniformity of density, impermeability to 25 water, malleability to resist wear and abrasion and certain elasticity. These qualities I have attained by the selection of materials and method of preparation of my block.

My process includes as one of its first 30 steps, the examination of the rock and of the asphalt contained in the asphalt rock as found.

I have found that certain rock in asphaltic rock deposits is capable of producing superior 35 block to those produced by other deposits.

The asphalt contained in the rock deposits is analyzed to determine its suitability for the purpose of making blocks for paving or other uses, and if found deficient in 40 certain essential qualities, these qualities are supplied by proper heating or addition of required rectifying materials, such as asphalt, dust, sand or oils or by the taking 45 away of certain detrimental elements or compounds.

In the block, I have made, I found that the asphalt contained in the rock deposit was of a suitable consistency and quality 50 if rectified by a certain grade of asphalt in small quantities. This was done by grinding the rock, heating and mixing while hot with the required amount of hot asphalt, then weighed and pressed into shape with 55 a hydraulic press. I have in this manner secured absolute density. Blocks that have been kept under water for three years have shown no signs of absorbing any water or of deterioration.

60 I have also examined other asphalt rock deposits, which in order to utilize successfully will be given a heat treatment, which it is possible to predetermine so as to produce a satisfactory block.

65 I have also produced block from another

deposit which on account of its mineral matter or rock produces a block of a quality less desirable for paving purposes, but more desirable for flooring.

Thus it can be seen that my process of utilizing asphalt rock for manufacturing pavements or blocks is different than any process heretofore utilized, and that one of the important steps in my process is the 70 analyzation of the rock deposit and predetermining the steps necessary for producing a satisfactory quality for the purpose to which the block will be used.

In all cases, where asphalt rock has heretofore been utilized, it was crushed to sizes 80 varying from one-half to three-fourths of an inch in diameter to powder, in other words, commonly known to the crushed stone trade as "crusher run." This is then spread out on the street and rolled or tamped. No effort has been made towards rectifying the asphaltic ingredients by quantity 85 or quality.

My purpose for finer grinding than this is two-fold. To secure an aggregate size better suited for paving purposes, and to secure 90 more uniformity in blending, thereby also resulting in a more uniform product.

The matter of compressing into blocks under great pressure secures a density which 95 it is impossible to secure by rolling or tamping.

Asphalt blocks as heretofore and now manufactured and used for paving purposes have not been made of mineral aggregates 100 under one-fourth of an inch and excluding the larger particles, nor have they been made of asphaltic rock pulverized and rectified as necessary.

I select natural asphaltic rock having an 105 asphaltic content of from four to twelve percentum.

The rock is ground, so that as used, substantially all of it should pass through a ten mesh screen and approximately ten 110 percentum or more should be of a size to pass through a two hundred mesh screen.

The mixture of ground rock is then heated to from two hundred to three hundred and fifty degrees Fahrenheit for melting 115 the asphalt and thoroughly diffusing it through the mass. The ground rock is preferably stirred or agitated during the heating to insure thorough mixing of particles to secure uniform density and homogeneity and proper diffusion of the asphalt. If it is desired to add more asphalt to the mixture, this is done while the mixture is hot. If it is desired to reduce the asphalt content, hot sand or mineral aggregate is 120 added to the mixture. The mixture is preferably weighed before being pressed, so that all blocks are of the same size and density.

While the mixture is hot, it is placed in 125

moulds and subjected to great pressure, as for example 7500 pounds to the square inch.

The product may be stored or shipped as soon as it has cooled.

5 By thus properly selecting the materials and processing the rock, there is secured a proper asphaltic content, mineral mixture and physical form for a proper product.

The product has been tested in pavement and affords a block having the desired qualities in high degree. The blocks in use have great strength and wear resistance, elasticity and malleability. The blocks do not break off at the edges but 15 give slightly until the joints between the blocks can scarcely be distinguished.

I claim as my invention:

1. An asphalt block comprising asphaltic rock with approximately four to twelve 20 percentum asphaltic content, of approximately fineness to pass a ten mesh screen with approximately ten percentum of a fineness to pass a two hundred mesh screen, mixed, heated and moulded while hot under great pressure.

2. The process of making asphalt blocks comprising the grinding of asphaltic rock of the asphaltic content of four to twelve percentum, till substantially all will pass a ten mesh screen and substantially one tenth will pass a two hundred mesh screen, mixing and heating the ground rock to a temperature of over two hundred and fifty degrees Fahrenheit and moulding the mixture under pressure of approximately seventy five hundred pounds to the square inch to the finished form.

3. The process of making asphalt blocks comprising the grinding of asphaltic rock of the asphaltic content of four to twelve percentum till substantially all will pass a ten mesh screen and substantially one tenth will pass a two hundred mesh screen, mixing and heating the ground rock to a temperature of over two hundred and fifty degrees Fahrenheit and moulding the mixture under great pressure.

Des Moines, Iowa, August 1, 1924.

MONROE LAWRENCE PATZIG.